

Dec. 26, 1933.

G. F. TAYLOR

1,941,283

DIAMOND DRILL AND METHOD OF MAKING THE SAME

Original Filed April 23, 1929

Fig. 1.



Fig. 3.



Fig. 2.



Fig. 4.



Inventor:  
George F. Taylor,  
by *Charles E. Tully*  
His Attorney.

## UNITED STATES PATENT OFFICE

1,941,283

DIAMOND DRILL AND METHOD OF MAKING  
THE SAMEGeorge F. Taylor, Schenectady, N. Y., assignor to  
General Electric Company, a corporation of  
New YorkApplication April 23, 1929, Serial No. 357,537  
Renewed January 29, 1931

9 Claims. (Cl. 76—108)

The present invention relates to diamond drills and the like. Heretofore such drills have been made by casting metal around spaced diamonds so that the diamonds protrude slightly from the metal matrix. When constructed in this manner however, the diamonds easily become loosened due to the great difference in the coefficient of expansion of diamond and the cast metal matrix. Even though the looseness is at first of a very small degree, it tends to increase very rapidly with any strain on the diamonds and finally results in the diamond cracking or becoming lost.

In my copending application Serial No. 357,536, filed April 23, 1929, and entitled "Abrading tools", I have disclosed and claimed a composition consisting of diamond particles and a binder material such for example as tungsten carbide and cobalt.

It is one of the objects of the present invention to provide a diamond drill in which the diamonds or cutting means are securely and permanently anchored in a sintered metallic matrix having a coefficient of expansion within the elastic deformation range of diamond, that is, the matrix can expand more or less with respect to the diamonds without causing the latter to become strained beyond their elastic limit.

The novel features which I believe to be characteristic of my invention are set forth with particularity in the appended claims. The invention itself however will best be understood from reference to the following specification when considered in connection with the accompanying drawing in which Fig. 1 is a view partly in section and partly in elevation of a mold whereby my invention may be carried into effect; Fig. 2 is a plan view of the lower portion of the mold; Fig. 3 is an exploded perspective view of the mold and a pressure applying member; while Fig. 4 is a perspective view, partly broken away, of a completed drill.

Referring more particularly to the drawing, I have indicated at 1 the bottom plate of a mold. The plate 1 has a recessed portion 2, a central countersunk portion 3, and a plurality of smaller countersunk portions 4 within which diamonds 4' may be positioned adjacent the periphery of the recess 2. The successive countersunk portions 4 are staggered so that alternate portions are located on the circumference of a circle having a diameter somewhat smaller than the diameter of recess 2, while the remaining portions are disposed on the circumference of a circle substantially equal to the diameter of recess 2 so that diamonds inserted therein will extend slightly

beyond the periphery of recess 2. The bottom plate 1 of the mold is made of carbon and provided with a pair of oppositely disposed upwardly projecting pins 5 adapted to engage cooperating openings 6 in the upper carbon plate 7 of the mold. Plate 7 is provided with a central opening 8 which is in alignment with recess 2 when plate 7 is so positioned on plate 1 that pins 5 engage the opening 6.

A carbon plug 9, which has a central projecting pin 10 adapted to engage the countersunk portion 3 of plate 1, extends through opening 8 and rests on the surface of recess 2 providing in this manner an annular or cylindrical space 11 between the plug 9 and the walls of opening 8 and recess 2, as clearly indicated in Fig. 1.

In manufacturing a drill according to my process, the diamonds are placed in the small countersunk portions 4 and the plate 7 and plug 9 properly positioned on plate 1. A powdered mixture consisting largely of tungsten-carbide but containing from 3 to 25% cobalt is then placed in the annular space 11 so that the powdered material extends substantially to a point adjacent the upper surface of the carbon plate 7. A carbon ring 12 is then inserted in the opening 11 and a pressure of about 1000 pounds per square inch applied to the upper end of the ring 12 while the powdered material is simultaneously heated to its sintering temperature by means of an electric current supplied to it through terminals 13 and 14 which may be clamped to the mold in any convenient manner. The mixed powdered materials are plastic at their sintering temperature and flow around the diamonds making intimate contact with them and holding them rigidly and permanently in position. The sintered annular matrix 15 may then be brazed, welded or secured in any suitable manner to a steel shank 16. The alternate diamonds 4' project inwardly and outwardly beyond the inner and outer circumferences of the sintered matrix 15. This arrangement requires that the carbon mold be broken in order to remove the matrix and attached diamonds therefrom. The cost of the carbon mold is relatively small and its loss therefore is of little consequence.

The powdered mixture employed to produce the metallic matrix is substantially the same as that disclosed in the patent to Schröter No. 1,549,615 and in general consists of a carbide of an element of the 6th group of Mendelejeff's periodic table and an auxiliary metal of the iron group, such as cobalt. Instead of a powdered mixture consisting of tungsten-carbide and cobalt, I may

employ a mixture consisting of the three elements tungsten, carbon and cobalt and sinter them under pressure in the same manner as the tungsten-carbide and cobalt.

5 In the present application the word "diamond" means a diamond of substantial size as distinguished from diamond powder. By the expression "spaced diamonds" I mean diamonds spaced out of contact with each other.

10 What I claim as new and desire to secure by Letters Patent of the United States, is:

1. A drill comprising a sintered, hollow cylindrical matrix, a plurality of spaced diamonds embedded in and protruding from the edge portion

15 of said matrix, said matrix consisting mainly of a carbide of a metal of the 6th group of Mendelejeff's periodic table.

2. A drill comprising a sintered, hollow cylindrical matrix, a plurality of spaced diamonds embedded in and protruding from the edge portion of said matrix, said matrix consisting mainly of tungsten-carbide but containing an appreciable amount of cobalt.

3. The method of forming a diamond cutting tool which comprises pressing a powdered mixture consisting largely of tungsten-carbide and cobalt around a plurality of spaced diamonds, while said powdered materials are heated to their sintering temperature.

30 4. A drill comprising a sintered hollow cylindrical matrix, a plurality of spaced diamonds embedded in and protruding from the edge portion of said matrix, said matrix consisting mainly of a carbide of a metal of the 6th group of Mendelejeff's periodic table but containing an ap-

preciable amount of metal of lower melting point than the carbide.

5. A drill comprising a sintered hollow cylindrical matrix, a plurality of spaced diamonds embedded in and protruding from the edge portion of said matrix, said matrix consisting mainly of tungsten carbide but containing an appreciable amount of metal of the iron group.

6. A diamond cutting tool consisting of a matrix and a plurality of diamonds embedded in and protruding from said matrix, substantially all of said diamonds being positioned in one plane, said matrix consisting of a cemented carbide.

7. A diamond cutting tool consisting of a matrix and a plurality of diamonds embedded in and protruding from said matrix, substantially all of said diamonds being positioned in one plane, said matrix consisting mainly of cemented tungsten carbide.

8. A diamond cutting tool consisting of a matrix and a plurality of diamonds embedded in and protruding from said matrix, substantially all of said diamonds being positioned in one plane, said matrix consisting of a sintered composition containing an appreciable amount of cobalt.

9. The method of setting diamonds or the like which comprises spacing a plurality of diamonds in a mold, applying to said diamonds a mixture of comminuted metallic material, which material has the property of closely adhering to said diamonds when heated to an elevated temperature and subsequently cooled, and then subjecting the mass to a temperature which does not impair the quality of said diamonds but is sufficiently high to sinter the mass into a coherent product.

113  
GEORGE F. TAYLOR.

40

115

45

120

50

125

55

130

60

135

65

140

70

145

75

150